

March 4, 1958

H. J. ROUX

2,825,660

WATERPROOF FIBERBOARD

Filed Dec. 30, 1954



INVENTOR  
HENRY J. ROUX

*by  
Henry J. Roux*

ATTORNEY

## 1

2,825,660

## WATERPROOF FIBERBOARD

Henry J. Roux, Lancaster, Pa., assignor to Armstrong Cork Company, Lancaster, Pa., a corporation of Pennsylvania

Application December 30, 1954, Serial No. 478,910

2 Claims. (Cl. 117—135.5)

This invention relates to a waterproof, vapor-permeable insulation board and method of producing the same, and more particularly to a conventional fiberboard insulation product having applied thereto a film of coating material which will resist the penetration of water into the board when exposed to rain but yet will not seal the board to such an extent that moisture from the interior of a building will be prevented from penetrating the board and passing through to the exterior.

In the construction of buildings, it has been common practice to apply a layer of insulating material such as "Temlok" sheathing on the exterior of the studding, forming the outer walls of the building. This sheathing is usually in place for a period of time before the exterior finish of the building is put in place over the sheathing. During this period of time, the sheathing is exposed to the weather; and if the material is not weatherproofed, the insulation becomes waterlogged and the insulating value is greatly diminished. In order to overcome this, it has been common practice to apply a film of asphalt to the surface of the sheathing material. This film of asphalt is waterproof and renders the sheathing resistant to rain when exposed to the elements; however, the asphalt coating is also vapor-impermeable, and thereby prevents the passage of moisture from the interior of the building through the insulating material to the outside of the building. This waterproof coating is applied to the outside of the insulating sheathing and, therefore, forms a vapor barrier at the outer surface of the sheathing, which means that the moisture condenses in the sheathing, thereby diminishing its insulating value. This has been overcome to a certain extent by applying a relatively hard asphalt coating, and depending on the heavy brittle coating, cracking upon drying, leaving small fissures through which moisture can escape. This is a rather haphazard arrangement, however, and the transmission of vapor through the fiberboard is diminished somewhat by this type of coating.

The invention set forth in this application is directed to a fiberboard material in which a film of asphalt emulsion and rubber latex, together with an alginate, is applied to the surface of the insulating board at the time the board is produced on a conventional web-forming fiberboard machine. This film of asphalt emulsion and rubber latex with the alginate renders the fiberboard resistant to water from the elements but renders the surface of the board vapor-permeable so that moisture transmitted from the interior of the building can pass freely through the fiberboard to the exterior. As a matter of fact, the transmission of the vapor through the board is not diminished to any appreciable extent because of the coating.

An object of this invention is to provide an insulating sheathing having applied thereto a waterproof, vapor-permeable coating which will render the insulation resistant to waterlogging caused from exterior water and will at the same time render the board vapor-permeable to permit the ready transmission of vapor through the board.

Another object of this invention is to provide a method

## 2

of producing a fiberboard with a waterproof, vapor-permeable coating by the application of a coating comprising asphalt emulsion, rubber latex, and an alginate at the wet end of the fiberboard forming machine.

5 In carrying out the invention, it has been found that soap type asphalt emulsion is best suited for producing the desired results. The rubber latex may be any of the conventional synthetic or natural rubber latices and the alginate may be any of the conventional commercially available alginates, such as, for example, "Keltex," which is a sodium derivative of algin and is one of the complex organic alginates.

I have found that a suitable formulation for carrying out the invention is as follows:

|    |                                                |       |
|----|------------------------------------------------|-------|
| 15 | <i>Example</i>                                 | Parts |
|    | Bitusize B (a soap type asphalt emulsion)      | 100   |
|    | Water                                          | 200   |
| 20 | Dow latex 512K (60% styrene and 40% butadiene) | 25    |
|    | "Keltex" (sodium derivative of alginate)       | 1.5   |
|    | Dowicide G (sodium salt of pentachlorophenol)  | 0.2   |

In the above formulation, the asphalt emulsion, which forms a major proportion of the coating, renders the coating water resistant and also helps to adhere the coating to the fiberboard. The latex 512K, which is a copolymer comprising 60% styrene and 40% butadiene, forms a coating for the asphalt particles. The rubber latex also aids in rendering the coating water repellent. While in the example given the rubber latex is a styrene-butadiene type latex, it will be understood that any of the conventional synthetic rubber latices or natural rubber latices are suitable for carrying out the invention. The rubber latex should be present in a quantity sufficient to coat the asphalt particles. The preferred range of rubber latex to asphalt emulsion has been found to be between .05 to .3 rubber latex compared to the quantity of asphalt emulsion used.

40 The "Keltex," which is a sodium derivative complex organic alginate, serves as a web for adhering the latex coated asphalt particles together. This forms a coating which is smooth but not continuous because of the extremely small interstices distributed uniformly throughout. These interstices are of such a nature that the water coming in contact with the exterior of the board will not penetrate the board through the interstices but the interstices permit vapor to pass therethrough as vapor pressure is built up in the board caused by vapor pressure differentials between the interior and the exterior of the board. For best results, the "Keltex" should be present in an amount ranging from .005 part to one part of asphalt emulsion to .01 part to one part of asphalt emulsion. The Dowicide G, which is a sodium salt of pentachlorophenol, is present as a preservative for the "Keltex" and the rubber latex. Any of the conventional preservatives for rubber latex are suitable for carrying out this purpose.

45 The attached drawing illustrates a piece of fiberboard with the waterproof vapor-permeable coating applied thereto.

In the application of the coating to the fiberboard, it has been found that the most expeditious way to apply the coating is to apply it at the wet end of the board-forming machine. When this is done, both the coating and the board can be dried simultaneously by one passage through the drier. If the coating is applied after the board has been formed and dried, it is necessary to utilize hot melt equipment on the application of a coating of asphalt to the surface of the board. The above coating could be applied to the dry board; however, an additional drying step would be involved and considerable

time and expense can be saved if the coating is applied at the wet end of the board-forming machine.

In the application of coatings at the wet end of the board-forming process, the problem of diffusion of the coating material through the wet board is of considerable importance. Most coatings applied at the wet end diffuse freely through the board and coat the fibers substantially uniformly throughout the board thickness. This is a costly proposition and requires a great deal more coating compound than is necessary to satisfactorily waterproof the board. It has been found by utilizing a coating of the type described herein a minimum of diffusion takes place because of the web structure which is formed by the alginic adhering the rubber-coated asphalt particles to one another. This weblike structure prevents undue diffusion into the board and the coating is merely applied to the surface of the wet board.

The coating is preferably applied to the wet board from a pool which is disposed back of a roller which engages the surface of the board with a slight amount of pressure. The wet board moves through under the reservoir of coating material and the excess coating material is removed by means of the roller which applies a slight amount of pressure to the surface of the wet board. After the board moves beyond the point at which the roller applies pressure, the board springs back to its original thickness and the thin film of coating material is applied uniformly to the surface of the board. This is only one of the many systems which may be utilized for the application of the coating composition to the board at the wet end of the board-forming machine. It will be understood that the coating material could be sprayed directly onto the finished web as it moves between the forming machine and the drier, and also the coating may be applied by means of a printing device coming in contact with the surface of the newly formed board as it is moving between the forming machine and the drier.

As the board is removed from the drying equipment, the surface is coated with a thin film of black coating material which renders the board waterproof; however, the coating does not diminish the transmission of vapor through the board to any appreciable extent.

I claim:

1. As an article of manufacture, an insulation board composed of matted and entangled fibers, said board having a normal heat insulating value and a coating adhering to said board to render said board waterproof and vapor-permeable without material diffusion of the coating into the interior of said board so as to alter substantially its normal heat insulating value and vapor permeability, said coating comprising a mixture of asphalt, rubber, and a water-soluble alginic.

2. As an article of manufacture, an insulation board composed of matted and entangled fibers, said board having a normal heat insulating value and a coating adhering to said board to render said board waterproof and vapor-permeable without material diffusion into the interior of said board so as not to alter substantially its normal heat insulating value and vapor permeability, said coating comprising a mixture of 100 parts asphalt, 10 to 30 parts rubber, and .05 to 2 parts of a water-soluble alginic.

References Cited in the file of this patent

UNITED STATES PATENTS

|    |           |             |               |
|----|-----------|-------------|---------------|
| 30 | 1,415,850 | Erdahl      | May 9, 1922   |
|    | 2,105,825 | Smith       | Jan. 18, 1938 |
|    | 2,210,348 | Swope       | Aug. 6, 1940  |
|    | 2,393,022 | Clark       | Jan. 15, 1946 |
|    | 2,701,219 | Fair        | Feb. 1, 1955  |
| 35 | 2,787,557 | Christensen | Apr. 2, 1957  |